

March 26, 1968

J. Y. WELSH

3,375,097

REDUCING TO MnO THE MnO<sub>2</sub> OF A MANGANESE ORE

Filed Oct. 18, 1965

3 Sheets-Sheet 1

Fig. 5.



Fig. 1.  
SCHEMATIC REPRESENTATION OF  
ZONES IN BED REDUCTION



INVENTOR  
JAY Y. WELSH  
BY Pierce, Schyffler & Parker  
ATTORNEYS

March 26, 1968

J. Y. WELSH

3,375,097

REDUCING TO MnO THE MnO<sub>2</sub> OF A MANGANESE ORE

Filed Oct. 18, 1965

3 Sheets-Sheet 2

*J.Y.W.*

ΔH OF AIR-METHANE REACTION FOR  
ONE MOLE OF METHANE AT INDICATED  
TEMPERATURES



INVENTOR

JAY Y. WELSH,

BY *Pierce, Schefler & Parker*

his ATTORNEYS

March 26, 1968

J. Y. WELSH

3,375,097

REDUCING TO  $MnO$  THE  $Mn_3O_4$  OF A MANGANESE ORE

Filed Oct. 18, 1965

3 Sheets-Sheet 3

*Fig. 2.*  
THEORETICAL ZONE I TEMPERATURE AS  
A FUNCTION OF AIR TO METHANE RATIO



*Fig. 3.*  
DH OF REDUCTION OF VARIOUS  
MANGANESE OXIDES TO PRODUCE  
TWO MOLES OF  $MnO$  AT 1800°F



INVENTOR

JAY Y. WELSH

BY Pierce, Scheffler & Parker  
his ATTORNEYS

1

**3,375,097**  
**REDUCING TO MnO THE MnO<sub>2</sub> OF A**  
**MANGANESE ORE**

Jay Y. Welsh, Catonsville, Md., assignor to Manganese Chemicals Corporation, Baltimore, Md., a corporation of Maryland

Filed Oct. 18, 1965, Ser. No. 496,965  
 12 Claims. (Cl. 75—1)

#### ABSTRACT OF THE DISCLOSURE

The higher oxide of manganese in a manganiferous ore material, in which the manganese values are present in the form of a higher oxide of manganese, is reduced to MnO by a method which comprises feeding an air-natural gas mixture (air ratio accurately controlled) through a hot bed of MnO<sub>2</sub>, and then causing the resulting gaseous products (which have a net reducing effect) to pass immediately into, and upwardly and outwardly through, a bed of the ore the surface of which bed is being fed with raw ore.

This invention relates to the art of reducing manganiferous ores in which the manganese values are present in the form of a higher oxide of manganese, and is particularly concerned with the reduction to MnO of the MnO<sub>2</sub> values of a manganese ore or ore material.

One of the most difficult problems encountered in the reduction of manganese ores has been the control of reaction heat. If a stable MnO product is desired—that is, a product which will not undergo reoxidation under ambient or near-ambient conditions—it is necessary that the reduction temperature be near or slightly above 1300° F. On the other hand, if the reduction temperature is about 2000° F. or higher the reducing ore may soften and bond together producing a "sinter" which is extremely difficult to handle or process. In an effort to circumvent the problem of temperature control, current reduction methods have become both expensive and troublesome.

It is an object of the present invention to provide a process by which the manganese ores comprising or consisting essentially of any normal oxide composition can be reduced in beds, piles or columns under precise temperature control and at a much lower cost than by current methods.

The basic principle of this process consists in feeding an accurately controlled ratio of air to hydrocarbonaceous gas (e.g., natural gas or methane) through a hot bed of MnO<sub>2</sub> and then causing the issuing gaseous products—having a net reducing effect—immediately to pass into and through a bed or layer of the raw manganese ore. It is apparent that these conditions are realized if the air-gas mixture is passed upwardly or outwardly through a bed of reducing ore, the surface of which is being fed with raw ore. Under these conditions the hot bed of MnO<sub>2</sub> is supplied by the ore which has undergone reduction and of course the issuing reducing gases from the MnO<sub>2</sub> bed pass directly into the raw ore layer on the surface of the MnO<sub>2</sub> bed. The hot bed of MnO<sub>2</sub> serves as a catalyst to promote a reaction between the air and the hydrocarbonaceous gas. MnO<sub>2</sub> is a very effective catalyst in this regard, and virtually any gas-air mixture can be made to react to its theoretical products even at temperatures as low as 700 to 800° F.

The advantages of this process over other methods can be fully understood only by a detailed discussion of the mechanical and thermodynamic factors involved. Such

2

a discussion will be shown in terms of a metallurgical grade pyrolusite ore containing 75% MnO<sub>2</sub> in its raw state and 84% MnO in its reduced state. The hydrocarbonaceous reducing gas will be considered as CH<sub>4</sub>, with CO and H<sub>2</sub> as special cases. The following discussion will refer to one or another of the appended drawings, in which:

FIG. 1 is a schematic representation of zones possibly existing in a manganese ore bed undergoing reduction;

FIG. 2 is a graph showing the heat of reaction of air and methane as a function of air-to-methane ratio and also as a function of temperature;

FIG. 3 is a graph showing the heat of reaction of higher oxides of manganese;

FIG. 4 is a curve correlating the heats of reaction with the heat capacity of the product gases, in terms of temperatures attained; and

FIG. 5 is a simplified diagrammatic representation of gases and solids flow in an ore bed.

In FIG. 1 various zones which can or do exist in a reducing ore bed are schematically indicated.

Case 1. As it stands FIG. 1 represents the zones ideally operating in the process of the present invention.

Case 2. If the reducing gas is methane only, zones I and II do not exist.

Case 3. If the primary reducing gas is either CO or H<sub>2</sub> (plus inert gases) or a combination of CO and H<sub>2</sub> instead of an air-methane mixture, zones I and II do not exist. Further, in the event of an excessive overblow of this reducing gas mixture zones IV and V are combined and zone VI is virtually non-existent.

FIG. 2 shows the heat of reaction of air and methane as a function of air to methane ratio, and also as a function of temperature. The 1500° F. curve represents the net heat of reaction taking place under the catalytic influence of MnO in zone I and III in a bed operating in proper thermal balance.

FIG. 3 shows the heat of reaction of MnO<sub>2</sub>, Mn<sub>2</sub>O<sub>3</sub> and Mn<sub>3</sub>O<sub>4</sub>, respectively with the gaseous products of the catalytic air-methane reaction, as a function of air-to-methane ratio. It is to be noted that the curves in both FIG. 2 and FIG. 3 show abrupt changes at an air-to-methane ratio of 2.4/1. This can be understood in terms of the products of the air-methane reaction at a temperature of 1500° F. or over. At a ratio of 2.4/1 the reaction products are essentially CO and H<sub>2</sub> only. Below a ratio of 2.4/1 increasing amounts of unreacted methane exist and above 2.4/1 increasing amounts of CO<sub>2</sub> and H<sub>2</sub>O are produced. In the case of FIG. 2 the high heat of formation of carbon dioxide and water account for the abrupt increase of heat of reaction above the 2.4/1 ratio. Applied to FIG. 2, the heat of reaction increases as the ratio of CO and H<sub>2</sub> to CH<sub>4</sub> increases. At the 2.4/1 ratio the reducing components remain CO and H<sub>2</sub> only, therefore the heat of reaction remains essentially the same.

Balancing the heats of reaction are four heat-consuming processes, viz:

(1) the heat required to raise the temperatures of the various gaseous components up to the temperatures existing in the bed;

(2) the heat required to raise the various solid components up to temperatures existing in the bed (the volatilization of free or chemical water contained in the ore is to be included in these values);

(3) the heat required to thermally decompose MnO<sub>2</sub> to Mn<sub>2</sub>O<sub>3</sub>; and

(4) heat removed from the system by radiation, convection, artificial cooling, etc.

In any bed process the above thermal processes must algebraically balance the reaction and gas transfer heats under steady state conditions, and—as mentioned previously—they must balance in such a way that the reduction zone temperature is controlled within the approximate temperature limits of about 1300 to 2000° F.

#### COMPARISON OF OTHER REDUCTION METHODS

##### A. Kiln

Before proceeding with a detailed discussion of bed, pile or column reduction systems, the reduction of ore in a rotating kiln will be considered for comparison. Basic in the operation of a kiln are the following features which distinguish from bed processes:

(1) The size of the ore particles must be small to permit complete reduction during the retention time of a kiln of practical length.

(2) A heat balance of the reacting materials does not have to be strictly maintained between the reactants themselves because heat can be artificially removed or added through the walls of the kiln to maintain the temperatures desired.

(3) Any movement of gas through the kiln in conjunction with a moving bed of finely divided solid material gives rise to the necessity of expensive dust collecting equipment.

(4) As opposed to bed reduction, coal or charcoal can be effectively used in kiln reduction providing an excess is employed.

(5) Expensive alloy tubes and troublesome mechanical maintenance are inherent.

(6) Gas permeability and heat transfer factors limit the depth of bed and tube size and therefore limit the rate of production per kiln.

It is apparent that the features characterizing kiln operation vs. bed operation are disadvantageous with possibly two exceptions, namely, the versatility with respect to heat balance and the ability to employ a solid fuel. Since the latter is often more expensive than natural gas and in addition leaves an undesirable residue, the option of its use is not attractive. And, since the proposed process provides a simple and practical method of controlling reaction temperatures (or heat balance) within a bed, kiln reduction methods appear to have no advantageous features.

##### B. Column reduction with producer gas

The reduction of a bed of ore with producer gas represents a special case of gas mixtures containing CO, H<sub>2</sub> and N<sub>2</sub>. The use of producer gas in bed reductions will be analyzed at this point for comparison also. A typical gas would be represented by the following composition:

|                              | Percent |
|------------------------------|---------|
| CO                           | 32      |
| H <sub>2</sub>               | 5       |
| CO <sub>2</sub>              | 2       |
| N <sub>2</sub> , (by volume) | 61      |

The gaseous reaction products will be:

|                  | Percent |
|------------------|---------|
| CO <sub>2</sub>  | 34      |
| H <sub>2</sub> O | 5       |
| N <sub>2</sub>   | 61      |

Consider a peak reaction zone temperature of 1860° F. The average mean heat capacity to this temperature is 0.0226 B.t.u./cu. ft. for the above product gases.

The reaction.—Mn<sub>2</sub>O<sub>3</sub>+2.7 (.32 CO+.05 H<sub>2</sub>) $\rightarrow$ 2 MnO 2.865 CO<sub>2</sub>+.135 H<sub>2</sub>O produces -41,400 B.t.u./# mole (2MnO).

The reaction.—2MnO<sub>2</sub>+5.4 (3.2 CO+.05 H<sub>2</sub>) $\rightarrow$ 2 MnO+1.73 CO<sub>2</sub>+.27 H<sub>2</sub>O produces -124,000 B.t.u./# mole (2MnO).

Heat Balance calculations: (based on 2 moles of MnO product)

| Input:                                                                                                              | B.t.u./# mole 2MnO |
|---------------------------------------------------------------------------------------------------------------------|--------------------|
| Heat transferred to cold ore by hot inert gas at 1860° F., based on the reduction of Mn <sub>2</sub> O <sub>3</sub> | -39,600            |
| Heat of reduction Mn <sub>2</sub> O <sub>3</sub>                                                                    | -41,400            |

Total transfer and reaction heat ----- -81,000

|                                                                                                     |        |
|-----------------------------------------------------------------------------------------------------|--------|
| Required:                                                                                           |        |
| Heat required to raise 2 moles of MnO as raw ore from 60° to 1860° F.                               | 28,600 |
| Heat required to thermally decompose 2MnO <sub>2</sub> to Mn <sub>2</sub> O <sub>3</sub> (1860° F.) | 34,400 |
| Heat required to raise 2 moles of MnO plus gangue from 60 to 1860° F.                               | 27,400 |
| Total heat required                                                                                 | 90,400 |

20 A similar calculation at a peak reaction temperature of 1360° F. gives:

| Input    | B.t.u. |
|----------|--------|
| Required | 68,600 |

25 Required ----- 77,900

These data indicate that a sufficiently high reaction temperature cannot be maintained if all of the MnO<sub>2</sub> is thermally decomposed to Mn<sub>2</sub>O<sub>3</sub> before the reduction takes place. In practice, however, the thermal decomposition reaction is not complete and net heat is added to the system in two ways, (1) from the direct reduction of a portion of the MnO<sub>2</sub> which produces (see reaction heat of the two reduction equations) about three times as much heat per unit of MnO produced as does the reduction of Mn<sub>2</sub>O<sub>3</sub>, and (2) by a corresponding reduction of the endothermic heat of decomposition of MnO<sub>2</sub> and Mn<sub>2</sub>O<sub>3</sub>. Fortunately, the proportion of MnO<sub>2</sub> undergoing thermal decomposition to the MnO<sub>2</sub> undergoing direct reduction is largely self-regulating. Thus, if the reaction zone temperature (zone IV, FIG. 1) is high, more heat will be transferred to the pre-heat and thermal decomposition zone (zone V, FIG. 1), giving rise to a greater degree of thermal decomposition. The converse is equally true.

30 40 45 50 55 Two factors effect the ability of the system to regulate itself in the manner described. (1) As the gas flow rate is increased, a point will be reached when increasing amounts of reducing gas will pass through the reduction zone and enter the pre-heat and thermal decomposition zone creating an ever widening intermediate zone labeled "zone (IV+V)" in FIG. 1. This in turn leads to an excessive proportion of direct MnO<sub>2</sub> reduction and excessive temperatures. (2) As the screen size of the ore is increased, both the rate of reduction and of thermal decomposition are decreased. The combined effect of these rate factors is again to broaden the intermediate zone (IV+V) and cause more direct reduction of MnO<sub>2</sub>, leading to excessive temperatures.

60 65 70 75 One extreme set of operating conditions should also be mentioned in connection with reduction of ore beds with producer gas. If very high gas flow rates are imposed, reaction zones IV and V (FIG. 1) merge into one composite zone and zone VI (FIG. 1) virtually disappears. Under these conditions the excessive heat of the direct MnO<sub>2</sub> reduction (which now comprises nearly 100% of the reduction processes) is removed from the top of the bed, thus permitting the temperature of the composite reaction zone to be controlled. This sheer brute force method requires about twice the amount of reducing gas.

It is apparent then that even though it is both feasible and practical to carry out the reduction of ore in a bed with producer gas, rather restrictive conditions must be imposed with respect to gas flow rate and/or ore particle size in order to avoid excessive temperatures within the ore bed. Further, producer gas inherently contains ob-

jectionable sulfur impurities as well as being unfavorable with respect to cost, convenience and maintenance. In the special case of ore containing oxygen corresponding to an  $Mn_3O_4$  level only, insufficient reaction heat is available even under the most favorable conditions to permit reduction by producer gas.

It will be shown in the subsequent heat balance analysis of ore reduction, by the use of air-methane mixtures that—unlike producer gas reduction—wide latitude is possible with respect to reduction rates (gas flow) as well as particle size range. Further, adjustments can be made which would even permit the reduction of ores containing manganese oxides at the  $Mn_3O_4$  oxidation level.

#### DISCUSSION OF PROPOSED PROCESS

As one varies the air-to-methane ratio two extremes of course are evident. As the air-to-gas ratio approaches 9.6/1 (the theoretical ratio for complete combustion) it is self-evident that bed temperatures will be excessive (over 3000° F.). In FIG. 2 and FIG. 4 it is readily apparent that air-to-gas ratios approaching 5/1 or even 4/1 would represent a practical upper limit, even zone I would approach or exceed 2000° F. The thermal characteristics of a reducing bed for which the air-to-gas ratio is zero (that is, pure methane) are not obvious and since this extreme has an important bearing on the overall concept, it will, in the following, be analyzed carefully and compared with experimental results.

A peak reaction zone temperature of 1860° F. and 100% direct reduction of  $MnO_2$  will be assumed. The average mean heat capacity of the  $CO_2$  and  $H_2O$  emerging from the reduction zone is 0.0255 B.t.u./cu. ft.

Heat balance calculations (based on 2 moles of  $MnO$  product)

| Input:                                    | B.t.u./mole (2MnO) |
|-------------------------------------------|--------------------|
| Heat transferred to cold ore zone=(.0255) |                    |
| (378)(1800) -----                         | 27,000             |
| Heat reduction -----                      | 58,300             |

Total heat conserved and produced .. 58,300

Required:

|                                                                                                                  |        |
|------------------------------------------------------------------------------------------------------------------|--------|
| Heat required to raise the raw ore and reactions products from 60° F. to 1860° F. raw ore from 60° F. to 860° F. | 45     |
| = (174/.75)(.16)(800) -----                                                                                      | 29,600 |
| $MnO$ plus gangue from 860° F. to 1860° F.=(142/.84)(.16)(100) -----                                             | 27,000 |
| Total heat required -----                                                                                        | 56,600 |

Thus, hypothetically, if 100% of the  $MnO_2$  were reduced directly by methane an excess of 85,300–56,600 or 28,700 B.t.u. of heat would be produced for each two moles of  $MnO$  product. The assumed temperature of 1860° F. could therefore not represent a stable condition and the reaction zone temperature would increase. Experimental data have shown the converse to be the actual result. In fact, if pure methane is used as the reducing gas the reduction zone temperature drops so low that the reduction can cease. The reason for this paradox has already been mentioned, namely, that the transfer of heat to the unreacted ore by the hot, inert gaseous reduction products is sufficient to thermally decompose a substantial portion of the  $MnO_2$  to  $Mn_2O_3$ . Calculations indicate that a theoretical balance would be reached if about 30% of the  $MnO_2$  thermally decomposed to  $Mn_2O_3$  before actual reduction took place, but since experiment indicates that a heat balance does not exist, appreciably more than 30% thermal decomposition must occur in the pre-heat and thermal decomposition zone (zone V, FIG. 1).

Accordingly, somewhere between an air-to-methane ratio of 0/1 and 4/1 there should exist a ratio of air-to-methane which gives the thermal balance required. This

has in fact been found to be true and, further, the range has been found to be sufficiently broad to render the process extremely practical. One of the reasons for a relatively broad range of operation has already been discussed in terms of the self-regulating control of the degree of thermal decomposition of  $MnO_2$  to  $Mn_2O_3$ . To the previous discussion in this regard one additional note should be added, namely, that a hot reduction zone not only transfers more heat to the thermal decomposition zone by virtue of the temperature of the issuing gases but also because there is a greater volume of them. That is, any  $MnO_2$  undergoing direct reduction, which is of course the source of the additional heat, also produces twice the volume of gaseous products as does  $Mn_2O_3$  per mole of  $MnO$  produced.

The air-to-methane ratio for reduction of a normal metallurgical pyrolusite ore by the present process has been found to fall within a range of about 2/1 to about 3.5/1. If exceptionally high production rates are desired per unit of bed surface or if exceptionally coarse ore is involved, ratios approaching 2/1 or even less may be required. The factors involved here have been discussed in connection with producer gas reduction. Conversely, low gas flow rates in conjunction with a finely divided ore or an ore with exceptionally low oxygen content may require air-to-methane ratios approaching 3.5/1 or even higher. Since an air-to-methane ratio of 2.4/1 falls well within the normal process range, and because of the simplicity of the equations involved, a complete thermal analysis will be made for this air-gas ratio. Conclusions concerning air-to-methane ratios falling on either side will be made when appropriate.

The reaction and heat effects taking place within the  $MnO$  zones, I, II and III (FIG. 1) are not only high relevant to the overall process but uniquely adapted to it. It has already been mentioned that  $MnO$  acts as a catalyst to promote air-methane reactions at low air-to-methane ratios and further will permit these reactions to take place at temperatures as low as 700 to 800° F. It is a very important ancillary fact that air-methane reactions can be established in a bed of  $MnO$  the temperature of which has fallen to as low as about 400° F. The process by which this is accomplished is two-fold in nature. (1) An air-to-methane ratio somewhat higher than normal should be chosen to reactivate such a cold  $MnO$  bed, a ratio of about 3.5/1 for example. (2) When the gas blow is started, the initiating reaction is between the air and the  $MnO$  since the catalytic air-methane reactions are largely inactive at temperatures as low as 400° F. The  $MnO$  reaction, however, produces heat which readily raises the advancing heat band to the temperature necessary to initiate the air-methane reactions; in fact, blowing air alone through such a bed can develop enough heat for fusion.

Once the catalytic air-methane reactions are initiated, no further oxidation of  $MnO$  will take place, and the reaction heat will be characteristic of the particular ratio. A 3.5/1 ratio of air-to-methane produces product gases at about 1550° F. (see FIG. 4). These gases as they move upwardly or outwardly through the bed will progressively bring the entire bed to 1550° F. level and will re-establish the reduction process if raw ore is placed on the surface. The air-methane ratio is then adjusted to a normal process level.

Thermodynamic analysis of the air-methane reactions taking place in zones I and III (FIG. 1) prove to be uniquely applicable to the process of the present invention. At an air ratio of 2.4/1, i.e.,  $\frac{1}{2}$  mole of  $O_2$  per mole of methane, the following reactions are possible:

- (1)  $CH_4 + \frac{1}{2} O_2 \rightarrow CO + 2 H_2$
- (2)  $CH_4 + \frac{1}{2} O_2 \rightarrow \frac{1}{2} CO_2 + H_2 + \frac{1}{2} CH_4$
- (3)  $CH_4 + \frac{1}{2} O_2 \rightarrow \frac{1}{2} C + H_2O + \frac{1}{2} CH_4$

A free energy analysis indicates that reaction (1) is very minor between 800 and 1000° F. and that reaction (3)

is somewhat predominant over reaction (2). At 1200° F. reactions (1), (2) and (3) are of about equal importance. At 1500° F. reactions (2) and (3) are both minor, and (1) is dominant.

FIG. 2 shows the heat produced by the above reactions (suitably weighted in accordance with their importance) as a function of air-to-methane ratio at various temperatures. The curve of FIG. 4 correlates the heats of reaction with the heat capacity of the product gases in terms of the temperature the product gases attain. The curve sections of FIG. 4 labeled A, B and C are of special significance to the reduction process under discussion. Curve section A is indicated as a solid line since the heat of reaction is dominated by reactions (2) and (3) which do not change appreciably in importance over the temperature range covered. Curve section B is indicated as a dotted line since it covers a temperature range which represents a transition from the dominance of reactions (2) and (3) to a dominance of reaction (1). Since the heat of reaction (1) is quite low—about  $\frac{1}{8}$  th that of reactions (2) and (3)—the curve falls off sharply below 1400° F.

Coincidental with the temperature level which permits the predominance of reaction (1) two additional (or sequential) reactions develop negative free energies and therefore take place:



Both reactions (4) and (5) have very high endothermic heats of reaction. These endothermic reactions proceeding concurrently (or predominately) from the products of reactions (2) and (3) stabilize the reaction gas temperature producing plateau line, section C. Beyond section C the excess  $\text{CO}_2$  and  $\text{H}_2\text{O}$  in the combustion products of the higher air-to-methane ratios cause a rapid rise in temperature of the resulting gaseous products.

Two additional reactions should be mentioned:



These reactions (6) and (7) both show negative free energy changes above about 1300° F., both are endothermic but less so than are (4) and (5).

These data can now be applied to zones I, II and III (FIG. 1). It is apparent from FIG. 4 that within the normal air-to-methane ratio range, the temperature in zone I is relatively constant at about 1250° to 1350° F. Further, since reactions (6) and (7) "go" within this temperature range, any carbon produced by reaction (3) is substantially removed from the surface of the ore particles. The temperature in zone II (1250° to 1350° F.) will maintain the same as the temperature generated in zone I. The gases moving through zone II are largely  $\text{CO}_2$ ,  $\text{H}_2\text{O}$  and unreacted  $\text{CH}_4$ .

In the specific case being analyzed, a 2.4/1 air-to-methane ratio, no extra reaction heat is available to cause endothermic reactions (4) and (5) to proceed. However, in zone III the air-methane reaction gases may encounter  $\text{MnO}$  higher in temperature. In fact the temperature of the upper part of zone III is very close to the temperature of the reduction zone, zone IV. Experimental measurements indicate zone IV may range in temperature from as low as 1200° to as much as 1900° F., depending on the rate of gas blow and the ore particle size. If a high zone IV temperature exists, the  $\text{MnO}$  in zone III represents a heat reservoir from which heat is supplied for the endothermic reactions (4) and (5). Calculations indicate that if the temperature drop between zone IV and zone II is 400° F. for higher, sufficient sensible heat will be supplied to complete reactions (4) and (5) before the reducing gases reach zone IV. Because of the endothermic reactions taking place, the temperature gradient in zone III (if one exists) will be relatively sharp. For the same reason the temperature of the gases entering

zone IV may be little above their temperature before entering zone III.

In zone IV active reduction of manganese oxides is taking place and reaction heat is produced. As indicated, zone IV may have a temperature range of 1200° to 1900° F. For the present analysis a temperature of 1800° F. will be used for the upper range and 1200° F. for the lower range. (A temperature as low as 1200° F. is extreme and would be avoided in practice.)

If as a first approximation it be assumed in both instances that  $\text{Mn}_2\text{O}_3$  is the only oxide undergoing reduction, then the reduction equation will be:



Input<sup>1</sup> (based on 2 moles of  $\text{MnO}$  produced):

<sup>1</sup>The average mean heat capacity of the product gases from 60 to 1800° F.=.0236 B.t.u. per cu. ft.

B.t.u./# mole  
(2MnO)

Heat transferred to zone V from zone IV by  
the hot product gases=(1740) (.0236)

(378) (1.63) ----- 25,300

Heat of reduction (FIG. 3) ----- 32,200

Total heat transferred and produced--- 57,500

Required:

Heat required to raise raw ore from 60 to  
860° F.=(174/.75) (.16) (800) ----- 29,800

Heat required to thermally decompose  
 $2\text{Mn}_2\text{O}_3$  ----- 34,400

Heat required to raise 2 moles of  $\text{MnO}$  plus  
gangue from 860 to 1800° F.=(142/.84)  
(.16) (940) ----- 25,400

Total heat required ----- 89,600

40 The calculations indicate that if all of the reduction in  
zone IV is based on  $\text{Mn}_2\text{O}_3$ , thermal balance cannot be  
maintained at 1800° F. The imbalance indicated is  
32,100 B.t.u. for each 2 moles of  $\text{MnO}$  less input than  
is required.

45 As a second approximation assume 25% of the prod-  
uct  $\text{MnO}$  is reduced in zone (IV+V), FIG. 1 from  
 $\text{Mn}_2\text{O}_3$ . The remaining 75% of the product  $\text{MnO}$  is as-  
sumed to be reduced in zone IV from  $\text{Mn}_2\text{O}_3$ .

The reduction equation of  $\text{MnO}_2$  is:



Input: B.t.u./# mole (2MnO)

Heat transferred to zone V from zones IV  
and (IV plus V)=(1740) (.0236) (378)

(1.63+X.25) ----- 31,600

Heat of reaction  $(-32,200 \times .75) + (-110 \times$   
 $000 \times .25)$  ----- 51,600

Total heat transferred and produced -- 83,200

60 Required:

Total heat required=89,600-(34,400)  
(.25) ----- 81,000

65 Thus, if slightly more than 75% of the  $\text{MnO}$  undergoes  
thermal decomposition in zone V and slightly less than  
25% still remains to be reduced directly in zone (IV plus  
V) a heat balance will be established.

70 *1200° F. case*

Input: B.t.u./# mole (2MnO)

Heat transferred by hot product gases ----- 19,000

Heat of reduction ----- 30,200

Total heat transferred and produced -- 49,200

|                                                                            |        |
|----------------------------------------------------------------------------|--------|
| Required:                                                                  |        |
| Heat to raise raw ore to 860° F. -----                                     | 29,800 |
| Heat to decompose MnO <sub>2</sub> to Mn <sub>2</sub> O <sub>3</sub> ----- | 34,400 |
| Heat to raise product MnO to 1200° F. -----                                | 9,200  |
| Total heat required -----                                                  | 73,400 |

In this instance the thermal deficiency is 24,200 B.t.u. instead of 32,100, and it would appear that about 19% of direct MnO<sub>2</sub> reduction is required to give a thermal balance.

The difference in the degree of thermal decomposition indicated above is obviously the reason for the low temperature of the reduction zone instead of the result. A higher (more efficient) degree of thermal decomposition occurs in the event of a low rate of gas blow in conjunction with a finely divided ore, which leads to low reduction zone temperatures. Further, the heat balance calculations for the 1200° F. case should be qualified. If the reduction zone is at 1200° F. no extra bed heat is available for endothermic reactions (4) and (5), and this heat must either be supplied by the reduction reaction (that is, more direct reduction of MnO<sub>2</sub> would be necessary than the 19% indicated, and such an indicated percentage may not exist) or by additional air in the air-methane mixture. In practice the latter is preferred (in fact is necessary for efficient operation). Thus, if a fine ore bed is to be reduced at a relatively low rate, higher air-to-methane ratios are needed, preferably sufficiently high to raise the reaction zone temperature to at least 1400° F.

Assume a reduction bed has been brought to a suitable thermal balance by an adjustment of the air-to-methane ratio. The proper ratio, as indicated, falls into a range either below 2.4/1 or above 2.4/1. At air-to-methane ratios between 2.4/1 and 2/1 little change will be observed in the conditions in zones I, II and III. The reduction heat generated in zone IV will drop significantly, however (see FIG. 3), thus compensating for a lower degree of thermal decomposition of MnO<sub>2</sub> to Mn<sub>2</sub>O<sub>3</sub>. At air-to-methane ratios less than 2/1 there will be a significant drop of the temperature in zone I with corresponding shifts up through the bed and a slight carbon deposit may also develop on the ore particles. Below an air-to-methane ratio of 1/1 the catalytic air-methane reaction will not function smoothly, and Mn<sub>3</sub>O<sub>4</sub> cycling may occur.

At air-to-methane ratios between 2.4/1 and slightly over 3/1, zones I and II will not change greatly with respect to temperature. However, more and more of the endothermic heat for reactions (4) and (5) will have been supplied by the air-methane reaction itself, zone III will be broader and the exit gases will pass into zone IV somewhat nearer to the zone IV temperature. Since the heat of reduction remains unchanged above the 2.4/1 ratio, it is apparent that the additional heat of the air-methane reaction compensates for the loss of reaction heat due to a greater degree of thermal decomposition of MnO<sub>2</sub> to Mn<sub>2</sub>O<sub>3</sub>. Above a ratio of 3.5/1 the temperature throughout the bed will rise rapidly and at about 4/1 even zones I, II and III will approach the limiting temperature of 2000° F. exclusive of the additional reduction heat. Gas-methane ratios within this range would be employed for ores very low in oxygen content.

*Additional notes.*—There are several comments (not included in the previous discussion) which are of importance:

(1) Of major importance is the fact that over one half of the reduction is carried out with hydrogen in the present process. This has an advantage when coarse ore is reduced since the rate of diffusion of hydrogen to the center of a lump of ore is about 3½ times that of carbon monoxide. The result is a narrower reduction zone and a more efficient heat interchange between zones IV and V. This fact in addition to the ability to adjust the heat of reduction downward by as much as 40% permits the re-

duction of coarse ore at high rates without danger of overheating.

(2) The gas entering the reduction zone contains a high percentage of reducibles: even the highest air-to-methane ratio of the normal operating range contains about 50% reducibles. This means relatively low gas flows per unit of production. High gas blows through an ore bed are generally undesirable because the fine ore particles are moved with the gas stream and tend to collect in pockets using poor gas distribution.

(3) The process once initiated in a proper bed is virtually 100% efficient with respect to methane utilization, and since some 75 to 80% of the reduction is from the Mn<sub>2</sub>O<sub>3</sub> level instead of from the MnO<sub>2</sub> level the process is very economical.

(4) The surface of the reacting bed is cool which minimizes operating hazards.

(5) The equilibrium temperature in the MnO bed due to the air-methane reaction is generally sufficient in itself to produce stable MnO regardless of the reduction zone temperature.

(6) It is normally desirable to limit the peak temperature to avoid partial fusion or "sintering." There are applications, however, for which partial fusion of an MnO product is desirable. It is important to note therefore that with higher air-to-methane ratios "sintering" can be produced, and—more important—that the degree of "sintering" can be controlled.

### Summary

Before proceeding with a discussion of types of reduction beds and the operational parameters involved, it is desirable to put the various factors which correlate with the proper choice of air-to-methane ratio in table form, as follows.

Factors which suggest a lower range of air to methane ratios:

- (1) Ore exceptionally high in MnO<sub>2</sub> content.
- (2) Ore with large mesh size.
- (3) High production (or, gas flow) rate.
- (4) Continuous processes in which all of the MnO corresponding to zones I and II (FIG. 1) is continuously removed.
- (5) Desirability of a reactive MnO.

Factors which suggest a higher range of air to methane ratios:

- (1) Ore with a high proportion of lower oxide.
- (2) Ore with low mesh size.
- (3) Low production (or, gas flow) rate.
- (4) Batch processing.
- (5) When a product is desired which is completely free from traces of carbon.
- (6) Exceptionally wet ore.
- (7) Desirability of very stable ore.

### APPLICATION OF PROCESS

#### Introduction

The versatility of the proposed method of reduction has been stressed and it will be evident that this versatility can be transposed to the type of equipment in which the reduction process is carried out. Since the problems of heat balance and temperature control within the reducing ore bed are inherently solved by the process itself, the design of equipment for an overall process is concerned almost entirely with three problems:

- (1) proper gas flow patterns within the bed;
- (2) suitable ore flow patterns (correlation between (1) and (2) is normally necessary); and
- (3) a means of cooling the product MnO subsequent to its participation in the reduction process.

The movement of gas through a finite ore bed is influenced by the following:

- (1) the container-bed interface. There is a marked tendency for higher gas flow rates at this interface than within the bed proper.
- (2) the distribution of the ore particle size within the bed. If the feeding pattern is such that particle size segregation occurs, the gas flow will tend to bypass areas containing a higher proportion of fines.
- (3) the temperature distribution in the bed. The gas flow, in terms of weight of gas per unit time, will tend to be highest through the colder areas of the bed.
- (4) the length of path. It is obvious but important that the highest flow of gas will tend to be through the shortest bed path.

#### Thermal stability of MnO in air

The stability of MnO in air will vary greatly depending upon the temperature at which it was reduced. Even the most stable MnO cannot be handled in an open system, however, unless it is first cooled to a suitable temperature level. In general, MnO should be cooled to at least 300° F. before exposure to an open atmosphere.

*Ore movement in a bin or cone.*—There is a marked tendency for any particulate material to flow much more rapidly from the center of the bin or cone than from the peripheral areas.

#### DISCUSSION OF VARIOUS TYPES OF ORE BEDS

##### Stationary

The most simple type of bed from the point of view of the operational parameters is a stationary one. For the process of the present invention, stationary beds offer several unique advantages. One special case, namely, of a simple pile on a flat surface, is of particular interest and will be discussed in detail.

#### PILE REDUCTION

Applications of the process of the present invention to reduction in a pile of ore requires only very simple and inexpensive apparatus, and is ideal for application to a manganese ore in the physical form in which it customarily moves in trade, namely, material varying in size from particles as large as one inch (or even larger) in diameter down through a progression of smaller and smaller sizes to fines. It is a batch process. It can be, and preferably is, carried out right on the ground. To prepare for carrying out the process a shallow hole is dug in the ground and in it a "distribution chamber" is constructed by placing on the earth "floor" of the hole bricks or blocks in two parallel rows and bridging the two rows with a row of bricks or blocks to form a grating over the distribution chamber. The bricks are laid up without mortar, and purposefully are spaced apart to provide plenty of interstices. An inlet pipe, partly buried in the ground, has its discharge end in this "distribution chamber" whilst its other, outer, end is branched and communicates with sources of a plurality of gases, as more specifically described hereinbelow. If a round pile of ore is to be built up, the distribution chamber and hole for the same are square or rectangular with the longer axis not very much longer than the shorter axis. If an elongated pile, or "windrow," of ore is to be built up the hole is an elongated ditch, and the distribution chamber within this ditch is correspondingly elongated. In either event, the hole is dug to such a depth that the top of the grating is at a level about opposite the level of the adjacent earth. Advantageously, a distribution chamber about eighteen inches in cross-section is adequate for an ore pile about twelve feet in cross-section.

To the branched outer end of the inlet pipe there are led a plurality of valved conduits leading, respectively,

from (1) a source of air under slight pressure, (2) a source of the selected hydrocarbonaceous fluid and (3) a source of an inert relatively cool cooling gas (which latter will be further described hereinafter).

To begin a batch operation, a small amount of the manganese ore material to be reduced is placed in a small pile over (e.g., on) the grating and heated to an elevated temperature (e.g., between about 800° F. and about 1200° F.) at which reduction of higher oxide of manganese to MnO proceeds at a desirable rate. This initial heating may be performed by burning in situ in the small pile of ore a combustible mixture of fluid fuel and air introduced into the ore by way of said distribution chamber. However, I prefer to effect this initial heating by forming the aforesaid small pile of ore about (i.e., over) a still smaller pile of charcoal lying on the aforesaid grating, lighting the charcoal, and blowing into the burning charcoal a controlled amount of combustion-supporting air (introduced by way of said distribution chamber) whilst slowly covering the pile of burning charcoal with successively applied individually very thin layers of the ore material. Application of ore to the pile advantageously is done, a shovelful at a time, by an operator who spreads out the shovelful over the top or over the sides of the pile in such thin layer.

It is an important feature of the process that the addition of ore material to the sides of the pile shall be in relatively thin layers and that the thin layer of ore be applied in such manner that the ore material cascades over a portion of a side of the pile, in order that the ore particles segregate (size-wise) at the pile surface, with the coarsest particles rolling faster and farther than the smaller particles whereby the particles adjacent the earth are relatively very coarse and hence their larger interstices influence ready passage of gases therethrough.

By the time the underlying charcoal has been consumed (burned), the covering of ore material will have "grown" so that a sizeable although still small pile of ore will have been formed. The layers of ore material overlying the burning charcoal tend to prevent complete combustion of the fuel, and the burning fuel gives off CO gas which—since it is hot and is an active reducing agent—in passing radially outwardly through the overlying ore heats the ore (thereby driving off the customarily present absorbed water) and raises its temperature to, say, 1000–1100° F. and simultaneously reduces the higher oxide of manganese present in the ore to MnO. Since this reduction is strongly exothermic, the temperature of the ore undergoing reduction usually rises to about 1700–1800° F. In consequence, a red-hot layer or zone of active reduction is maintained only a few inches beneath the surface of the pile, and the gases moving radially outwardly through this highly heated layer carry the heat along into the outermost layers of fresh ore material.

As soon as there has been formed a sizeable but still small pile of ore material in the interior of which reduction is taking place, the operator feeds to the aforesaid distribution chamber a stream of gaseous mixture containing a gaseous carbonaceous fuel. Advantageously, this mixture may be a mixture of natural gas rich in methane,  $\text{CH}_4$  (and hereinafter sometimes referred to simply as "methane"), and air, in controlled amounts relative to each other and in an aggregate amount controlled with due regard to the rate of progress of reduction in the ore pile. Since hot MnO is an active cracking agent the air-natural gas mixture as it becomes heated by contact with hot ore is cracked to a mixed gas—reducing in net effect—consisting essentially of CO,  $\text{H}_2$ ,  $\text{CO}_2$  and  $\text{N}_2$  (together with some uncracked  $\text{CH}_4$ ). The relative amounts of air and natural gas thus mixed and cracked are adjusted to about the ratio of 3-to-1. During the building up of the pile the operator uses a thermocouple stuck into the pile to determine the temperature pattern, and adjusts the relative amounts of natural gas

and air to maintain relatively constant the previously stated temperature zones. If the ore is very high grade, the ratio may be altered in the direction of a 2:1 ratio, whereas when the ore contains much gangue or an unusual amount of absorbed water the air-natural gas ratio may be altered in the direction of a 4:1 ratio.

As was mentioned above, the ore is so delivered onto the sides of the pile as to induce segregation of particles to bring it about the particles nearest the ground are the largest particles of the ore. Whilst continuing to furnish the aforesaid mixed gas of net reducing effect the operator continues to add ore—in the manner above described—the additions being made with strict regard to the temperature distribution pattern within the ore pile. This temperature pattern can—in effect—be visually ascertained, in the sense that wherever the radially outwardly moving gas mixture finds a zone of readiest egress that zone will become highly heated fastest and the zone of maximum temperature within the pile will lie nearest the exterior surface of the pile. Since the waste gases exiting from the pile contain much water vapor, the pile “steams” visually. Those spots on the surface where the emerging steam is the densest are the hottest spots. Whenever and wherever the operator sees an unevenness in the density of the emerging steam he feeds layers of ore to such a “hot spot” at an enhanced rate and until the denseness of steam emanating from such “hot spot” has become the same as that in the areas surrounding such spot. In the ideal situation, steam emanates from the pile at a uniform intensity throughout the entire surface of the pile. Since conditions are never “ideal” for any length of time, the operator keeps watch over the steaming pile and applies his next shovelful or so where more steam is seen. In other words, he “feeds (ore) to the hot spots.”

All during this procedure, the natural gas and air entering the pile from the distribution chamber quickly become highly heated by the hot reduced ore which the mixture first contacts, and the mixture is cracked to a reducing gas mixture of CO, H<sub>2</sub>, CO<sub>2</sub>, N<sub>2</sub> and some uncracked CH<sub>4</sub>. Simultaneously with the cracking, the gases are highly heated to about or above 1000° F. These hot reducing gases pass radially outwardly, through the pile, into the overlying layer of highly heated unreduced ore which they encounter and drive off water from, and heat, and reduce the same to MnO. With proper operation the gases actually emerge from the exterior surface of the pile containing no or only a little CO or H<sub>2</sub>, and simply are water vapor, carbon dioxide and nitrogen.

The reduction which proceeds radially outwardly as the pile “grows” occurs in a layer which is only two or three inches, under the actual surface of the pile: if the operator pushes the ore away with the tip of his shovel he can see the red-hot layer of the “fresh” ore just under the surface.

As the pile of ore continues to grow, it inherently changes its general shape, and becomes less and less “spread out” over the ground. When the angle of the layer under-going active reduction (or, differently expressed, where the angle of the zone of maximum temperature) has reached the steepness of the angle of repose of the ore, it is time to stop feeding ore to the pile. The product pile at this stage consists of the ore with a thin “skin” (outermost layer) of unreduced or incompletely reduced ore on the surface. Continuance of ore feed would simply bring it about that the heat pattern no longer could be followed with the ore pattern and the base of the ore layers would be too thick to reduce. In a one-man operation this stage may be reached in about 20 hours. However, the operator continues to supply natural gas through the distribution chamber for some time (say, one-half hour) after he has stopped feeding ore to the sides of the pile, whereby to provide enough reducing gas to finish the reduction of the final outer layer of ore. Just as soon as

that has been accomplished, he substitutes for the natural gas a cooling gas non-oxidizing towards MnO which is passed radially outwardly through the pile, from the distribution chamber, until the whole body of ore has been cooled down to a temperature at which the MnO of the reduced ore will not reoxidize in the presence of air. As soon as this has been accomplished, the batch process is at an end, and the reduced ore can be picked up (e.g., with a power shovel) and moved to a point of further use. Then the batch procedure may be repeated.

10 The above-mentioned “cooling gas” may be any gas which is non-oxidizing to MnO. Thus, it may be room-temperature nitrogen or carbon dioxide from any suitable source. In lieu thereof, a cool reducing gas such as CH<sub>4</sub>, 15 CO, H<sub>2</sub>, etc. probably could be used. Advantageously, an operable cool neutral gas economically may be produced at the site by (1) burning natural gas in an amount of air yielding oxygen in a stoichiometric amount with respect to the combustibles content of the natural gas, 20 thereby producing a “neutral gas,” and (2) cooling the combustion gases as, for example, by passing said gases through a water spray, and then blowing the so-cooled inert gas through the aforesaid inlet pipe and into and through said distribution chamber into and through the 25 reduced ore pile. Presumably, steam might be used as cooling agent although steam does re-oxidize a small proportion of the MnO. The worst aspect of cooling with steam is that steam hydrates the MnO—once it has cooled down to a lower temperature near the boiling point of 30 water—and the manganese hydrate is unstable in air, even at room temperature. Accordingly, steam is not an industrially feasible cooling agent in this connection.

It is believed that the process is operable using crushed ore material of any normal size distribution (e.g., with 35 the largest lumps not larger than 2-3 inches in diameter and the greater part falling within the minus 1/2 inch-fines range). Presumably, it would not be economically feasible to crush finer than all minus one-half inch. Crushing in a jaw crusher gives a desirable particle size distribution (not too large a proportion of fines).

#### SPECIFIC EXAMPLE

In one specific reduction to practice of the process of the present invention, applicant used a manganese ore which, as received, had been crushed to minus three-eighths inch diameter, which material contained particles in all sizes down to (and including considerable) fines. It analyzed 48-50% Mn, mostly as MnO<sub>2</sub>, with the remainder being the usual gangue constituents Al<sub>2</sub>O<sub>3</sub>, SiO<sub>2</sub>, Fe<sub>2</sub>O<sub>3</sub>, H<sub>2</sub>O and alkaline and alkaline earth metal oxides. 50 This material could not be reduced in a shaft-type reduction apparatus because the considerable amount of fines in the material created an intolerably high back pressure; nor could it be reduced in an indirectly heated reduction tube furnace of practical length and normal feed rate, 55 because some of the material was too coarse. As will appear, applicant's reduction process successfully handled a raw material which neither of the present-day “conventional” processes could tolerate.

60 In this instance when using the above ore, and working with a round pile (of ore) over a distribution chamber about 48 inches by 18 inches by four inches, the operator fed through the distribution chamber about 25 c.f.m. of natural gas and 75 c.f.m. of air. The temperature maintained in the zone of reduced ore was 1300-1400° F., and in the zone of active reduction (the red-hot layer only an inch or so beneath the exterior surface of the pile) the temperature was about 1800° F. The operator progressively fed fresh ore, shovelful-by-shovelful, to the 65 dry (hot) spots to maintain a uniform heat pattern and uniform diffusion (steaming) pattern. The end of the growth of the pile was reached when about 17 tons of fresh ore had been fed to it: at that stage, the height of the pile was about 4.5 feet and the sides of the pile were at 70 the angle of repose of the ore. The operator stopped feed- 75

ing ore after 19 hours, and then continued to feed the gas mixture for about one (1) hour. Cool gaseous combustion products (derived from burning natural gas with a neutral flame and cooling by passing the gaseous combustion products through a water spray) were then passed into the distribution chamber and from thence radially through the bed. This cooling step was continued until the temperature of the ore was lowered to a point, e.g., about 300° F., at which the ore was stable in air.

In all, the batch required about 50 hours.

The material in the so-treated pile was sampled in an approved manner and was analyzed for its content of  $Mn_2O_3$  and  $MnO_2$ . The material two inches and more below the surface was found to contain none of its manganese values in a state of oxidation higher than  $MnO$ .

The identical process can be operated employing an elongated "windrow" type of pile, over a correspondingly elongated distribution chamber.

If producer gas were used in lieu of natural gas, the reduction might be carried out without adding air (or other oxidizing gas); however, by so doing one would lose the great economic advantage resulting from cracking the natural gas-air mixture in situ in the hot reduced ore. On the other hand, if one were to generate  $CO$ , only, in situ within the pile by blasting burning coal with air, the resulting very high temperature of combustion would fuze everything in the immediate vicinity whilst underheating the outer portions of the pile, with resulting formation of extensive masses of clinker worth less than nothing.

The process of the present invention, as practiced on manganese ore, is attended by a further economic advantage, as follows: The customary uses or applications of  $MnO$  (i.e., of reduced manganese ore) call for a finely ground product, e.g., 98% minus 200 mesh. In the conventional tube furnace process the ore is crushed, ground to final size, and finally reduced. According to the present process the ore is only coarsely crushed (e.g., to all minus three-eighths inch) and then reduced and finally ground to desired final size. The reduced ore is relatively very friable, and hence is a great deal easier to grind than is the raw ore. The difference in grinding costs is very significant.

Relative to reduction in the pile, the following qualifications and additions should be mentioned:

(a) All of the bed zones which have been discussed hereinabove, along with the corresponding interplay of chemical reactions, are applicable to pile reduction; also, the changes in thermal balance as a function of gas velocities and ore particle size.

(b) Special consideration must be given to the change of gas velocities through the reduction and preheat zones in the case of pile reduction. If a constant gas-air feed is introduced into a pile, it is evident that as the pile grows in size the gas flow per unit area through the outer zones decreases. In accordance with the preceding discussions, the ratio of air to methane should increase accordingly, in order to preserve a suitable reaction zone temperature. An alternate, of course, is to correlate the gas flow rate with the surface area. In practice it is generally more convenient to change the gas-air ratio than the gas feed rate.

(c) The segregation of ore fed to the side of the pile (as described under "Pile Reduction" above) is much more pronounced as the upper screen size of the ore is increased. The limiting cross section of a pile, therefore, increases as a direct function of the ore particle size.

#### Cone reduction

Certain advantages can be realized if a batch reduction is carried out in a cone-shaped vessel (see FIG. 5).

(a) A body of the ore contained in an inverted cone-shaped vessel 10 with sides 11 at about a 65° angle with respect to the horizontal has a gas flow pattern such that a flat reaction surface is developed, i.e., the rate of gas flow per unit surface 12 is nearly uniform over a

horizontal plane surface at any vertical level within the cone. This offers a simplification with respect to feeding the raw ore.

Other parts of the structure indicated in FIG. 5 include the following: At its apex 13 the vessel 10 projects into a catalyzer which latter may (as is suggested in the drawing) take an inverted cone form 15 akin to the form of vessel 10. The top 16 of the catalyzer has an opening 18 into which the apex outlet 20 of vessel 10 projects, said top having a horizontal dimension such that particulate solids gravitationally descending from vessel 10 into catalyzer 15 can take an angle of repose directly beneath the top or "roof" of 15, leaving above the angle of repose a free space 19 into which an air-methane gas mixture may be introduced via conduit means 21.

Catalyzer 15 is superimposed above a cooling vessel 25, and particulate solids gravitationally descending from catalyzer 15 into cooler 25 make this transition out of access of air, the apex discharge outlet 26 of catalyzer 15 having an air-tight fit with an opening 27 in the upper surface of cooler 25.

(b) Once the cone 10 is filled to the desired level the reaction is allowed to proceed to the ore surface 12 and the reduced  $MnO$  can be drawn off through any type of conventional controlled atmospheric cooling mechanism as suggested at 25. In practice a heel of the hot  $MnO$  is left in the bottom of the cone which provides the catalytic zone for a fresh batch reaction.

#### Moving or continuous beds

If the  $MnO$  is drawn off continuously from the cone just described, then a mechanical compensation must be made for the fact that the gas flow pattern does not correlate with the ore flow pattern. The rate of reduction, as pointed out above, is essentially uniform over the entire (flat) surface of the bed while the ore tends to move down through the center. If new raw ore were fed to the center only, to replace the ore withdrawn, the reducing gas emerging through the outer areas of the bed would not be productive and the reducing gas emerging through the center area would be insufficient to reduce the raw ore fed.

One solution to this problem is to feed raw ore to the periphery of the bed only and progressively to move it toward the center by a series of simple rotating plows. This procedure is illustrated in simple embodiment in FIG. 5 wherein at the upper right hand edge of vessel 10 there is suggested the raw ore be fed to the periphery of the charge bed and be gradually swept inward (over the bed) toward the center of the bed's surface. This permits productive utilization of the reducing gas emerging over the entire surface of the bed while at the same time compensating for the uniform ore flow.

I claim:

1. Process of reducing to  $MnO$  the content of higher oxides of manganese in a manganese ore, which comprises passing a methane-rich hydrocarbonaceous gas-air mixture, in which the ratio of air to methane is within the range of about 2:1 and about 4:1, into and through a body of reduced manganese ore whose oxide of manganese content is in the form of  $MnO$ , said reduced ore being at an elevated temperature of from about 1000° F. to about 2000° F., whereby to form in the gaseous mixture a substantial content of active reducing gas including  $CO$  and  $H_2$ , and passing the resulting hot reducing gas-containing mixture into and through a layer of initially unreduced manganese ore contiguous to said body of reduced ore whereby to reduce to  $MnO$  the higher oxides of manganese in said layer.

2. Process of reducing to  $MnO$  the content of higher oxides of manganese in a manganese ore, which comprises passing a methane-rich hydrocarbonaceous gas-air mixture, in which the air-methane ratio is from about 2.4:1 to about 3.5:1, into and through a body of reduced manganese ore whose oxide of manganese content is in

the form of MnO, said reduced ore being at an elevated temperature of from about 1250° to about 1350° F., whereby to form in the gaseous mixture a substantial content of active reducing gas including hydrogen and CO, passing the resulting hot reducing gas-containing gaseous mixture into and through a layer of initially unreduced manganese ore contiguous to said body of reduced ore whereby to enlarge the body of reduced ore, and thereafter cooling reduced ore in that part of said body which is remote from said layer to a temperature at which MnO is relatively stable by passing therethrough a current of relatively cool non-oxidizing gas.

3. Process of reducing to MnO the content of higher oxides of manganese in a manganese ore, which comprises passing a methane-rich hydrocarbonaceous gas-air mixture, in which the air-methane ratio is from about 2.0:1 to about 4.0:1, into and through a body of reduced manganese ore whose oxide of manganese content is in the form of MnO, said reduced ore being at an elevated temperature of from about 1250° to about 1350° F., whereby to form in the gaseous mixture a substantial content of active reducing gas including hydrogen and CO, passing the resulting hot reducing gas-containing gaseous mixture into and through a layer of initially unreduced manganese ore contiguous to said body of reduced ore thereby enlarging the body of reduced ore and to develop a zone of maximum temperature.

4. The process defined in claim 2, in which the ratio of air to methane is so adjusted within the range 2.0-4.0:1 as to maintain the temperature within the layer wherein reduction of higher oxide of manganese to MnO is progressing within the range 1300°-2000° F.

5. The process defined in claim 4, in which said body is progressively enlarged by successive additions of fresh layers of unreduced ore to said body as the higher oxide content of the ore in the underlying layers becomes reduced to MnO.

6. The process defined in claim 5, in which the size of said body is maintained within predetermined limits by progressively withdrawing reduced ore from said body in amounts equivalent to the amounts of unreduced ore added to said body.

7. Process of reducing a manganese ore whose manganese content is mostly in the form of a higher oxide of Mn which ore is substantially free from pieces larger than 3 inches in diameter and has a normal size distribution, which process comprises

establishing a gas distribution chamber covered by a grating; forming a small initial pile of the ore on top of the grating covering said chamber; heating the small initial pile of ore with heating gases passing outwardly from the vicinity of the chamber by burning a carbonaceous fuel with air adjacent said chamber, the heating being continued until at least the interior of said initial pile has attained a temperature of at least 800° F.;

progressively feeding ore in relatively thin layers to the top and to the sides of the pile in a manner to establish and maintain a substantially uniform temperature pattern over the peripheral portion of the pile while

simultaneously outwardly passing through the pile from adjacent said distribution chamber a reducing gas mixture rich in CO and H<sub>2</sub> whereby to create and maintain a zone of active reduction of the higher oxide of manganese to MnO;

continuing the passage of said reducing gas mixture while continuing feeding of the ore to maintain substantially uniform the thickness of the layer of relatively unreduced ore exterior to the zone of active reduction,

the ore being fed to the top and to the sides of the pile in cascading thin layers and in a manner which in-

5

10

15

20

25

30

35

40

45

50

55

60

65

70

75

duces particle size segregation as the ore cascades over the surfaces of the pile;

terminating the feeding of ore when it no longer is possible to maintain substantial uniformity in the thickness of the layer of unreduced ore exterior to the zone of active reduction;

substituting a relatively cool non-oxidizing gas for the reducing gas whereby to cool the material of the pile from the center outwardly, and continuing such passage of said relatively cool non-oxidizing gas until the temperature of substantially all of the material of the pile has been lowered to a temperature at which the reduced material is substantially stable to air.

8. Process of reducing a manganese ore whose manganese content is mostly in the form of a higher oxide of Mn which ore is substantially free from pieces larger than 3 inches in diameter and has a normal size distribution, which process comprises

establishing a gas distribution chamber covered by a grating;

forming a small initial pile of the ore on top of the grating covering said chamber;

heating the small initial pile of ore with heating gases passing outwardly from the vicinity of the chamber by burning a carbonaceous fuel with air adjacent said chamber, the heating being continued until at least the interior of said initial pile has attained a temperature of at least 800° F.;

progressively feeding ore in relatively thin layers to the top and to the sides of the pile in a manner to establish and maintain a substantially uniform temperature pattern over the peripheral portion of the pile while

simultaneously outwardly passing through the pile from adjacent said distribution chamber a reducing gas mixture rich in CO and H<sub>2</sub> whereby to create and maintain a zone of active reduction of the higher oxide of manganese to MnO;

continuing the passage of said reducing gas mixture while continuing feeding of the ore to maintain substantially uniform the thickness of the layer of relatively unreduced ore exterior to the zone of active reduction,

the ore being fed to the top and to the sides of the pile in cascading thin layers and in a manner which induces particle size segregation as the ore cascades over the surfaces of the pile;

terminating the feeding of ore when it no longer is possible to maintain substantial uniformity in the thickness of the layer of unreduced ore exterior to the zone of active reduction;

continuing the passage of reducing gas until the aforementioned unreduced ore layer has been substantially reduced;

substituting a relatively cool inert gas for the reducing gas whereby to cool the material of the pile from the center outwardly, and continuing such passage of said relatively cool inert gas until the temperature of substantially all of the material of the pile has been lowered to a temperature at which the reduced material is substantially stable in air.

9. The process defined in claim 8, in which the reducing gas mixture is produced in situ within said pile by catalytically cracking an air-natural gas mixture introduced into the pile by way of said distribution chamber.

10. The process defined in claim 9, in which the zone of catalytic cracking is maintained at from about 1250° to about 1400° F., while the zone of active reduction is maintained at from about 1400° to about 1900° F.

11. The process defined in claim 8, in which the relatively cool inert gas consists essentially of non-reducing gaseous products of the combustion of natural gas in a stoichiometrically equivalent amount of air.

12. Process of reducing to MnO the content of higher oxides of manganese in a manganese-containing material the manganese content of which is in the form of oxides whose oxygen contents lie between  $Mn_2O_3$  and MnO, which comprises passing a methane-rich hydrocarbonaceous gas-air mixture, in which the air-methane ratio is from about 3:1 to about 5:1, into and through a body of reduced manganese-containing material whose manganese content is in the form of MnO, said reduced material being at an elevated temperature of from about 1400° to about 1800° F., whereby to form in the gaseous mixture a substantial content of active reducing gas including hydrogen and CO, passing the resulting hot reducing gas-containing gaseous mixture into and through a layer of said

5

manganese-containing material in initially unreduced form said layer being contiguous to said body of reduced manganese-containing material thereby enlarging the body of reduced manganese-containing material.

10

manganese-containing material in initially unreduced form said layer being contiguous to said body of reduced manganese-containing material thereby enlarging the body of reduced manganese-containing material.

## References Cited

## UNITED STATES PATENTS

|           |        |                      |        |
|-----------|--------|----------------------|--------|
| 1,951,342 | 3/1934 | Bradley et al. ----- | 23—145 |
| 2,310,258 | 2/1943 | Riveroll -----       | 75—80  |
| 2,745,730 | 5/1956 | De Vaney -----       | 75—1   |
| 3,149,961 | 9/1964 | Moklebust -----      | 75—80  |

BENJAMIN HENKIN, Primary Examiner.

DAVID L. RECK, Examiner.